

# United States Patent Office

3,272,622

Patented Sept. 13, 1966

1

3,272,622

## HIGH HEAT RESISTANT STEELS

Karl-Inge Bengtsson, Koping, Sweden, assignor to Aktiebolaget Bofors, Bofors, Sweden, a corporation of Sweden

No Drawing. Continuation of application Ser. No. 686,556, Sept. 27, 1957. This application Aug. 29, 1962, Ser. No. 220,160

Claims priority, application Sweden, Sept. 29, 1956,

8,890/56

1 Claim. (Cl. 75—126)

This application is a continuation of my pending application, Serial No. 686,556, filed September 27, 1957, now abandoned.

The present invention relates to alloy steels with a high resistance. In particular it is directed to alloy steel intended preferably for use in the production of tools with very severe requirements for high heat resistance.

The tools aforesaid are forging tools, hot-pressing tools, die-casting tools, and extrusion tools. Certain of those tools can attain temperatures of between 900 and 1000° C. when in use. As it is not possible for these tools to hold the said temperatures, they must be cooled down discontinuously with water, or in some other way, to temperatures of approximately 500°. The said cooling takes place very rapidly, and therefore the requirements stipulated for the alloy used are very severe.

Hitherto, alloys of, e.g. the following compositions have been used:

### ANALYSIS

| Steel No. | C    | Si   | Cr  | Mo  | W   | V    |
|-----------|------|------|-----|-----|-----|------|
| I         | 0.30 | 0.30 | 3   | —   | 9   | 0.30 |
| II        | 0.30 | 0.30 | 1   | —   | 5.5 | 0.2  |
| III       | 0.45 | 0.30 | 1.5 | 0.7 | —   | 0.3  |
| IV        | 0.40 | —    | 5   | 1.5 | —   | 1    |
| V         | 0.30 | 0.3  | 12  | —   | 12  | 0.5  |

The hot hardness of the above-mentioned steels has been determined with the aid of a Vickers diamond at the temperatures 600°, 650°, 700° and 750° C. All of the test pieces of the alloys have been hardened and tempered at 600° C. before the hardness testing. A summary of the hardness values is given in the following table:

### HOT HARDNESS D.P.H.

| Steel No. | 600° C. | 650° C. | 700° C. | 750° C. |
|-----------|---------|---------|---------|---------|
| I         | 290     | 187     | 113     | 70      |
| II        | 272     | 197     | 127     | 75      |
| III       | 235     | 163     | 105     | 62      |
| IV        | 312     | 205     | 108     | 67      |
| V         | 276     | 232     | 180     | 137     |

The heat resistance of the above-mentioned alloys is determined by the alloy elements, of which different alloys have different properties that raise the heat resistance. As a rule, the greater the content of the alloying element, the greater heat resistance is obtained. Most alloys, however, have the disadvantage that the greater the quantity of alloying element used, the poorer the heat-conducting properties of the alloy. The poorer the heat-conducting properties, the greater the risk for cracking on rapid cooling of a tool made of the alloy.

Of the above-mentioned five alloys, it has proved that all of them are sensitive to cracking when cooled, but to different degrees. Thus, steel V is the one most sensitive to heat checking; thereafter in the order mentioned: steels I, IV, II and III.

The above-mentioned known steels can also contain

2

quantities of one or more of the alloys titanium, columbium and tantalum, with contents of up to 0.5%.

In the above-mentioned alloys it is known to vary the relation between the alloys contained in them, so that alloys with greater heat-resistance-raising properties dominate the alloy, a high heat resistance thus being obtained with as small a quantity of alloying elements as possible, in order to obtain high heat resistance, at the same time as good heat-conducting properties are obtained.

It is one of the principal objects of the present invention to provide a new alloy of the last-mentioned kind, i.e., with a low content of alloying elements and high heat resistance. A further object is to provide novel articles, such as tools, etc., made from such novel steel.

15 The steel of this invention is characterized by its containing, 0.20-0.40% carbon; 0.2-0.5% of silicon; 2-3% of chromium; 2-3% of molybdenum; 0.3-0.6% of vanadium; and 2-3% of cobalt; and in addition, normal contents of the basic elements usually occurring in steels.

20 Within this invention is an alloy steel with a high heat resistance characterized by the feature that it contains as alloying elements: 0.28-0.32% carbon, 0.20-0.35% Si, 2.6-3.0% Cr, 2.6-3.0% Mo, 2.6-3.0% Co and 0.45-0.55% V, the remainder being principally iron.

25 The alloy according to this invention can also contain one or more of the alloys titanium, columbium and tantalum, in contents of up to 0.5%.

The following are examples in accordance with this invention.

### Example I

A steel alloy is made according to this invention which has the following composition (in percent by weight) of alloying elements:

### ANALYSIS

| Steel No. | C    | Si   | Cr   | Mo   | V    | Co   |
|-----------|------|------|------|------|------|------|
| VI        | 0.29 | 0.37 | 2.89 | 2.66 | 0.41 | 2.75 |

The steel has the following hot hardness:

| Steel No. | 600° C. | Hot hardness,<br>650° C. | D.P.H. at<br>700° C. | 750° C. |
|-----------|---------|--------------------------|----------------------|---------|
| VI        | 350     | 225                      | 137                  | 75      |

45 This steel has proved to be superior to all hitherto known steels tested for which high heat resistance requirements are severe; and which at the same time must be capable of withstanding sudden cooling.

### Example 2

A steel is made in accordance with this invention which has the following composition:

|    | Percent |
|----|---------|
| C  | 0.28    |
| Si | 0.24    |
| Cr | 2.6     |
| W  | 5.2     |
| V  | 0.50    |
| Co | 2.72    |

65 It will be understood that the foregoing description of the invention and the example set forth are merely illustrative of the principles thereof. Accordingly the appended claim is to be construed as defining the invention within the full spirit and scope thereof.

What is claimed is:

70 An alloy steel with a high heat resistance characterized by the feature that it consists essentially of: 0.28-0.32% carbon, 0.20-0.35% Si, 2.6-3.0% Cr, 2.6-3.0% Mo,

2.6-3.0% Co and 0.45-0.55% V, balance essentially iron.

References Cited by the Examiner

UNITED STATES PATENTS

1,496,980 6/1924 Armstrong ----- 75-128 X  
1,545,094 7/1925 Giles ----- 75-128 X  
2,289,449 7/1942 Nelson ----- 75-126

FOREIGN PATENTS

377,011 7/1932 Great Britain.  
404,565 1/1934 Great Britain.

<sup>5</sup> DAVID L. RECK, *Primary Examiner.*  
P. WEINSTEIN, *Assistant Examiner.*